# EUROPEAN PATENT SPECIFICATION

(11) **EP 2 256 228 B1**
(45) Date of publication and mention of the grant of the patent: **11.10.2017**
(21) Application number: 10158900.0
(22) Date of filing: 31.03.2010
(51) Int. Cl.: C23C 4/12, C23C 28/00, C23C 28/04

(54) **Layered coating for erosion protection**
Lagenbeschichtung zum Erosionsschutz
Couche stratifiée pour la protection contre l'érosion

(30) Priority: 27.05.2009 US 472871
(43) Date of publication of application: 01.12.2010
(73) Proprietor: United Technologies Corporation, Farmington, CT 06032 (US)
(72) Inventor: Nardi, Aaron T., East Granby, CT 06026 (US); Shi, Jun, Glastonbury, CT 06033 (US); Smith, Blair A., South Windsor, 06074 (US)
(74) Representative: Hall, Matthew Benjamin

(56) References cited:
- EP-A1- 0 526 670
- EP-A1- 1 980 645
- DE-A1-102004 032 342
- UTSUMI ET AL: "Effect of a hard supra-thick interlayer on adhesion of DLC film prepared with PBIID process" NUCLEAR INSTRUMENTS & METHODS IN PHYSICS RESEARCH, SECTION - B:BEAM INTERACTIONS WITH MATERIALS AND ATOMS, vol. 257, no. 1-2, 1 April 2007 (2007-04-01), pages 706-709, XP022014801 ELSEVIER, AMSTERDAM, NL ISSN: 0168-583X DOI: 10.1016/J.NIMB.2007.01.127
- SHANOV V ET AL: "CVD diamond coating for erosion protection at elevated temperatures" JOURNAL OF MATERIALS ENGINEERING AND PERFORMANCE, vol. 11, no. 2, April 2002 (2002-04), pages 220-225, XP002607210 ASM INTERNATIONAL, US DOI: 10.1361/105994902770344303

## Description

The present invention relates to a layered coating sheath for erosion protection of metal parts that are subjected to erosive forces of particulate such as sand, dirt and dust, or liquid impingement such as rain or other fluids.

Layered wear coatings are known in various fields, for example DE 10 2004 032 342 discloses a two-layer low-friction wear coating for a piston, comprising a lower carbide layer on which is formed an upper CrN layer. An article titled "Effect of a hard supra-thick interlayer on adhesion of DLC film prepared with PBIID process" and published in Nuclear Instruments and Methods in Physics Research, vol., 257, no. 1-2, discloses a further high wear, low-friction coating having a diamond-like carbon (DLC) outer layer and a metallic interlayer of tungsten-carbide to improve adhesion of the DLC layer.

Erosion of components of aircraft propulsion systems such as rotor blades, propeller blades, fan blades and fan inlet cases, is an issue that has continued to be a source of problems for the industry. Other industries where fluid handling or air handling equipment can be subject to particulate or fluid impingement suffer from similar issues. These might include wind or water turbines, impellers, sea vessel propellers, or large commercial piping systems. Of particular concern is erosion caused by sand, because sand typically contains a wide range of particle sizes. Sand may contain particles as small as 20 to 30 microns and as large as 1,000 to 2,000 microns. Finer sand tends to produce slow abrasive wear with little impact energy keeping the depth of effected material low. Fluids can also produce damaging results if impinged upon the substrate in a repetitive manner. In this case again larger fluid droplets at higher velocity can produce high stresses deep into the material. On helicopters for instance, the leading edge of the rotor blade may be fitted with an abrasion strip or sheath, often fabricated from titanium and/or nickel. These blades are subjected to severe erosion, especially on takeoff and landing in a desert location or in severe rain.

Sheathing has been used in the past to address erosion problems on erosion prone equipment such as those previously mentioned. Sheathing often consists of nickel, cobalt, titanium, nickel-cobalt alloy, or in some cases elastomers to resist the erosion. Materials used for sheathing need to be tough with high strain to failure values or need to be able to absorb high amounts of energy without damage accumulation to perform well in high incident angle erosion. These materials need high hardness and abrasion resistance to resist erosion at low angles of incidence.

Thin ceramic layers like titanium nitride tend to spall when used on traditional sheath materials like nickel. Cermets, or ceramic materials held together by a metal matrix, such as tungsten carbide-cobalt can have a higher overall hardness than much of the naturally occurring particulate found in erosive environments. Additionally, these materials may be able to absorb some of the impact energy due to the more ductile matrix material. This leads to a coating that may perform generally well with very little surface deformation occurring. This same coating can however fail from erosion of the softer metal between the carbide particles, which then allows the carbide particles themselves to become dislodged. Some layers of erosion protection materials like these are effective against one range of particle size and not against a different range of particle size. Nothing has been found to cover the whole range of particle sizes that are encountered in many environments. Similarly rain or fluid erosion may be able to damage the softer matrix or may propagate matrix damage caused by particulate erosion.

The present invention provides a coating for protecting a surface against erosion when contacted by particles having a range of particle sizes (such as sand having a particle size ranging from about 20 microns to about 2000 microns) or by repetitive high velocity fluid impingement (such as water or other fluid impinging the component repetitively with high velocity), consisting of: a first coating sufficiently high in bulk composite hardness to resist deformation from particles or fluid impact pressure, wherein the first coating is a cermet; and a second continuously hard coating on the first coating having a hardness higher than the first coating and the hardness of the particles, the second coating being a ceramic layer selected from the group consisting of titanium nitride, diamond, chrome nitride, diamond-like-carbon, cubic boron nitride, boron carbide, titanium carbide, or a combination of these.

The first layer is relatively hard, such as having a hardness of from about 10 to about 20 Gigapascals, and is relatively thick, such as from about 75 to 500 microns. The second layer is much harder, such as from about 19 to about 40 Gigapascals or higher, and is relatively thin, such as from about 1 to about 25 microns. The function of the first, thicker layer is to provide resistance to penetration by particles on impact sufficiently to minimize large surface deformations that cause thin coating spallation and debonding. The second, thinner layer resists abrasion of the softer metal matrix of the first layer. The first thicker layer may be formed, for example, from tungsten-carbide-cobalt, tungsten-carbide-cobalt-chrome, chrome-earbide-nickel-chrome, chrome-carbide-nickel, diamond-nickel, or other metal matrix materials with ceramic reinforcement. The second thin layer is formed from titanium nitride, diamond, chrome nitride, diamond-like-carbon, cubic boron nitride, boron carbide, titanium carbide, or a combination of these or other high hardness ceramic thin coatings. Since hardness is often measured with a diamond, it is difficult to have a precise value for the maximum hardness for this layer, but the minimum value should at least exceed the maximum possible hardness of any particulate erodent expected.

Certain preferred embodiments of the present invention will now be described in greater detail and by way of example only with reference to the accompanying drawings, in which:
FIG. 1 is a schematic view of a surface protected by the layered coating of the present invention;
FIGS. 2A and 2B are photographs of the surface of a test strip with a first layer of this invention with a CVD diamond second layer material similar to the concept of FIGURE 1, before and after the surface has been subjected to erosion with sand;
FIGS. 3A and 3B are photographs of a titanium metal which is softer than the first layer of Figs 2A and 2B with a CVD diamond second layer applied, before and after the surface has been subjected to erosion with sand; and
FIGS. 4A and 4B are photographs of the surface of a test strip with a first layer with a chromium nitride second layer material applied, before and after the surface has been subjected to erosion with sand.

A coating is provided to protect a surface against erosion when contacted by particles such as sand, dirt and the like, particularly when the particles have a range in particle size. The first coating is applied to form a deformation resistant surface that has a composite hardness exceeding that of the erodent expected but is a composite of hard materials with a softer ductile matrix to absorb energy. The second coating is applied to the first coating with a hardness higher than the first coating, but also with a hardness consistent across the surface.

FIG. 1 illustrates the erosion protection system 10 for protecting a substrate 11 that has a relatively low hardness such that it would be eroded by contact with erosion particles 13 and 15 that are of different particle sizes. Sand, for example, can range in particle size from less than 20 microns to more than 2,000 microns. Erosion protection system 10 also is effective against particles of a generally similar size. Substrate 11 represents any surface that is exposed to erosion. For example, titanium and nickel are two surfaces that are used in leading edges of helicopter rotors. They are strong for their intended purpose but they erode and require frequent repair or replacement.

Surface 11 is first covered with a high bulk hardness coating 17 that is relatively thick, such as from about 75 to about 500 microns thick. Coating 17 thickness can also range from 100 to 300 microns. Cernets, which are composites of very hard ceramic particles or fibers in a matrix of a more ductile metal combine the properties of ceramic and metallic materials, and form coatings that may be used for coating 17. Examples are tungsten-carbide-cobalt, tungsten-carbide-cobalt-chrome, chrome-carbide-nickel-chrome, chrome-carbide-nickel, diamond-nickel, or other metal matrix materials with ceramic reinforcement. The hardness of coating 17 ranges from about 10 to about 20 Gigapascals. This hardness should vary dependent on the hardness of the erodent expected in service. For instance for an environment dominated by erosion by silica, a more narrow range of about 15 to about 18 Gigapascals may be used.

The high bulk hardness coating 17 is then coated with a hard coating 19 that is much harder than coating 17, and is also much thinner. Coating 19 may range in thickness from less than 1 micron to more than 25 microns. Thicknesses from about 2 to about 15 microns, and more particularly about 3 to 10 microns have proven very effective. Coating 19 is a ceramic coating, and should have a hardness ranging from about 18 to about 40 Gigapascals or higher. Examples of such ceramic coatings are titanium nitride, diamond, chrome nitride, diamond-like-carbon, cubic boron nitride, boron carbide, titanium carbide, or a combination of these or other high hardness ceramic thin coatings. A narrower range is from about 18 to about 30 Gigapascals.

Coating 17 may be applied to substrate 11 by HVOF, cold spray or other processes used for applying a cermet on to a substrate. Coating 19 is applied to first coating 17 by chemical vapor deposition or physical vapor deposition, and by other methods of applying a thin ceramic coating to a surface.

In order to demonstrate the efficacy of the present invention, a number of tests were performed to compare the coatings of this invention with other coatings. Test strips were prepared and subjected to Ottawa sand impacting on the surface of the strip at an angle of 90° and with a velocity of 800 feet/second (244 meters/second).

Fig. 2A is a photograph of a chemical vapor deposited diamond coating on a tungsten carbide-cobalt coating. Fig. 2B is a photograph of the test strip of Fig. 2A after being hit by 500g of sand. As can be seen, there is essentially no erosion of the coating.

Fig. 3A is a photograph of the same chemical vapor deposited diamond coating on a soft titanium alloy such as the alloys used as a leading edge protector on a helicopter rotor blade. Thus this sample does not have the high bulk hardness coating of the invention. Fig. 3B illustrates the sample after only 2g of sand impacting under the same test conditions. Clearly the protective diamond film has been removed from the surface and will erode at the relatively high titanium erosion rate.

Fig. 4A is a photograph of a chrome nitride layer that has been applied with physical vapor deposition on a tungsten carbide-cobalt coating. Fig 4B illustrates the sample after 100g of sand has hit it, which is a fifty percent improvement.
Presented below in Table I are sand erosion test results performed on titanium and nickel abrasion strips currently used on helicopter rotor blades, again with Ottawa sand impacting at 90° impact and at a speed of 800 feet/second (244 meters/second). The values are based on an uncoated nickel or titanium value of 1.0.

**TABLE I**

| Thin film coating | Substrate or bulk hardness coating | Improvement Relative to Nickel | Improvement Relative to Titanium |
|---|---|---|---|
| Diamond | Tungsten carbide with 6% cobalt | 3851 | 8003 |
| Diamond | Titanium | 0.45 | 0.93 |
| Chrome Nitride | Tungsten carbide with 10% cobalt | 18 | 37 |

As can be seen, the use of a thin film coating with the high bulk hardness coating of this invention provides substantial improvement in erosion resistance, similar to that shown in Figs. 2A, 2B, 4A, 4B.

The erosion protection system of the present invention may be used on helicopter rotor blades, propellers, land-based turbines, power generators, and fan blades on turbine engines, as well on any surface that is subjected to particle erosion, liquid impingement erosion, or a combination of the two.

Although the present invention has been described with reference to preferred embodiments, workers skilled in the art will recognize that changes may be made in form and detail without departing from the scope of the invention, which is defined by the claims.

## Claims

1. A coating (10) for protecting a surface (11) against erosion when contacted by particles having a range of particle sizes or by repetitive high velocity fluid impingement, consisting of:
a first coating (17) sufficiently high in bulk composite hardness to resist deformation from particles or fluid impact pressure, wherein the first coating (17) is a cermet; and
a second continuously hard coating (19) on the first coating having a hardness higher than the first coating and the hardness of the particles, the second coating being a ceramic layer selected from the group consisting of titanium nitride, diamond, chrome nitride, diamond-like-carbon, cubic boron nitride, boron carbide, titanium carbide, or a combination of these.

2. The coating of claim 1, wherein the cermet is selected from the group consisting of tungsten-carbide-cobalt, tungsten-carbide-cobalt-chrome, chrome-carbide-nickel-chrome, chrome-carbide-nickel, diamond-nickel, or other metal matrix materials with ceramic reinforcement.

3. The coating of any preceding claim, wherein the first coating (17) has a thickness from about 75 to 500 microns.

4. The coating of any preceding claim, wherein the first coating (17) has a hardness of from about 10 to about 20 Gigapascals.

5. The coating of any preceding claim, wherein the second coating (19) has a thickness from about 1 to about 25 microns.

6. The coating of any preceding claim, wherein the second coating (19) has a hardness from about 18 to about 40 Gigapascals.

7. A component of an aircraft propulsion system, the component comprising:
a substrate (11), and a protective coating as claimed in any preceding claim on the surface of the substrate.

## Patentansprüche

1. Beschichtung (10) zum Schützen einer Oberfläche (11) gegen Erosion, wenn sie mit Partikeln unterschiedlicher Partikelgröße in Kontakt tritt, oder bei wiederholtem Auftreffen von Fluid mit hoher Geschwindigkeit, bestehend aus:
einer ersten Beschichtung (17) mit einer ausreichend hohen Grundverbundwerkstoffhärte, um einer Verformung durch Partikel oder Fluidaufpralldruck zu widerstehen, wobei die erste Beschichtung (17) ein Cermet ist; und
einer zweiten durchgehend harten Beschichtung (19) auf der ersten Beschichtung mit einer höheren Härte als die erste Beschichtung und als die Härte der Partikel, wobei die zweite Beschichtung eine keramische Lage ist, ausgewählt aus der Gruppe bestehend aus Titannitrid, Diamant, Chromnitrid, diamantartigem Kohlenstoff, kubischem Bornitrid, Borcarbid, Titancarbid oder einer Kombination davon.

2. Beschichtung nach Anspruch 1, wobei das Cermet aus der Gruppe bestehend aus Wolframcarbid-Kobalt, Wolframcarbid-Kobalt-Chrom, Chromcarbid-Nickel-Chrom, Chromcarbid-Nickel, Diamant-Nickel oder anderen Metallmatrixmaterialien mit Keramikverstärkung ausgewählt ist.

3. Beschichtung nach einem der vorhergehenden Ansprüche, wobei die erste Beschichtung (17) eine Dicke von etwa 75 bis 500 Mikrometern aufweist.

4. Beschichtung nach einem der vorhergehenden Ansprüche, wobei die erste Beschichtung (17) eine Härte von etwa 10 bis etwa 20 Gigapascal aufweist.

5. Beschichtung nach einem der vorhergehenden Ansprüche, wobei die zweite Beschichtung (19) eine Dicke von etwa 1 bis etwa 25 Mikrometern aufweist.

6. Beschichtung nach einem der vorhergehenden Ansprüche, wobei die zweite Beschichtung (19) eine Härte von etwa 18 bis etwa 40 Gigapascal aufweist.

7. Komponente eines Flugzeugantriebssystems, wobei die Komponente Folgendes umfasst:
ein Substrat (11) und eine Schutzbeschichtung nach einem der vorhergehenden Ansprüche auf der Oberfläche des Substrats.

## Revendications

1. Couche (10) pour la protection d'une surface (11) contre l'érosion lorsqu'elle entre en contact avec des particules ayant une fourchette de taille de particules ou par impact répétitif de fluide à haute vitesse, composée :
d'une première couche (17) avec une dureté composite globale suffisamment élevée pour résister à la déformation provoquée par la pression de l'impact de particules ou de fluide, dans laquelle la première couche (17) est un cermet ; et
une seconde couche continuellement dure (19) au-dessus de la première couche ayant une dureté plus élevée que la première couche et la dureté des particules, la seconde couche étant une couche de céramique choisie dans le groupe composé de nitrure de titane, de diamant, de nitrure de chrome, de carbone de type diamant, de nitrure de bore cubique, de carbure de bore, de carbure de titane, ou d'une combinaison de ceux-ci.

2. Couche de la revendication 1, dans laquelle le cermet est choisi dans le groupe composé du tungstène-carbure-cobalt, du tungstène-carbure-cobalt-chrome, du chrome-carbure-nickel-chrome, du chrome-carbure-nickel, du diamant-nickel, ou d'autres matériaux de matrice métallique avec un renforcement céramique.

3. Couche d'une quelconque revendication précédente, dans laquelle la première couche (17) a une épaisseur allant d'environ 75 à 500 microns.

4. Couche d'une quelconque revendication précédente, dans laquelle la première couche (17) a une dureté allant d'environ 10 à 20 gigapascals.

5. Couche d'une quelconque revendication précédente, dans laquelle la seconde couche (19) a une épaisseur allant d'environ 1 à environ 25 microns.

6. Couche d'une quelconque revendication précédente, dans laquelle la seconde couche (19) a une dureté allant d'environ 18 à environ 40 gigapascals.

7. Composant d'un système de propulsion d'un avion, le composant comprenant :
un substrat (11), et une couche protectrice selon une quelconque revendication précédente sur la surface du substrat.
